

[54] PYROLYtic COATINGS OF  
MOLYBDENUM SULFIDE BY PLASMA  
JET TECHNIQUE

[72] Inventor: Ting Li Chu, Dallas, Tex.

[73] Assignee: Westinghouse Electric Corporation, Pittsburgh, Pa.

[22] Filed: Nov. 5, 1968

[21] Appl. No.: 773,537

## Related U.S. Application Data

[62] Division of Ser. No. 483,670, Aug. 30, 1965, abandoned.

[52] U.S. Cl.....117/93.1 PF, 117/105.2, 117/121,  
117/127, 252/31, 23/206

[51] Int. Cl.....B05b 7/22

[58] Field of Search .....117/93.1 PF, 46 FS, 105, 105.1,  
117/105.2; 23/206, 208, 209.1, 209.4, 209.3;  
204/174; 252/25, 31

[56]

## References Cited

## UNITED STATES PATENTS

|           |         |                     |             |
|-----------|---------|---------------------|-------------|
| 2,922,869 | 1/1960  | Giannini et al..... | 117/93.1 PF |
| 2,960,594 | 11/1960 | Thorpe.....         | 117/93.1 PF |
| 3,246,114 | 4/1966  | Matvay.....         | 117/93.1 PF |
| 3,275,408 | 9/1966  | Winterburn .....    | 117/105.2   |

|           |         |                  |             |
|-----------|---------|------------------|-------------|
| 3,331,664 | 7/1967  | Jordan .....     | 23/209.3    |
| 3,346,338 | 10/1967 | Latham.....      | 23/208 A    |
| 3,411,949 | 11/1968 | Hough.....       | 117/93.1 PF |
| 3,458,341 | 7/1969  | Diefendorf.....  | 23/209.4    |
| 3,485,591 | 12/1969 | Evans et al..... | 23/208 A    |
| 3,503,787 | 3/1970  | Pendse .....     | 117/93.1 PF |

## FOREIGN PATENTS OR APPLICATIONS

863,190 3/1961 Great Britain.....117/93.1 PF

## OTHER PUBLICATIONS

Davis " Metal Progress" Vol. 83 No. 3 March 1963 pp. 105-108, 142, 144, 146, 148

Primary Examiner—Alfred L. Leavitt

Assistant Examiner—J. H. Newsome

Attorney—F. Shapoe and C. L. Menzemer

[57]

## ABSTRACT

A plasma-forming fluid consisting of a monatomic gas and at least one other gas having a diatomic molecule is employed to pyrolytically produce chemical elements and chemical compounds, such, for example, as pyrolytic carbon and refractory carbides. Pyrolytic carbon having a density of from 2.1 to 2.25 grams per cubic centimeter and an impurity content of less than 20 parts per million is made from a reactant material comprising aliphatic halides of carbon introduced into the plasma-forming fluid.

1 Claim, 3 Drawing Figures

Patented April 25, 1972

3,658,572



FIG. 2.



FIG. 3.

**PYROLYTIC COATINGS OF MOLYBDENUM SULFIDE  
BY PLASMA JET TECHNIQUE**

**CROSS-REFERENCES TO RELATED APPLICATION**

This patent application is a division of my copending application Ser. No. 483,670, filed on Aug. 30, 1965 now abandoned.

This invention relates to pyrolytic coatings of chemical elements and chemical compounds and methods of producing the same by plasma jet techniques.

The plasma jet technique has been used for the plating and coating of various chemical elements and compounds onto suitable substrates. For instance, the coating of objects, which will be subjected to extreme thermal conditions, with refractory materials is well known. The plasma jet plating technique has also been used for the fabrication of semiconductor devices to provide ohmic contacts and junctions.

In the conventional jet plating technique, the chemical element or compound, usually in the powder form, is introduced into a plasma jet where it receives energy by collisions with the plasma particles. The plasma jet then transports the element or compound involved to the substrate surface at high directed velocities and it is deposited as a coherent and adherent coating upon the suitable substrate. The density and uniformity of the coating depends upon many factors such as the enthalpy of the plasma jet and the physical properties of the material being deposited, such as melting point, particle size, the rate and uniformity of its introduction into the plasma jet stream and the like. Unless the material being deposited is melted, or finely dispersed, in the plasma jet, the deposited material usually has a density lower than its true density and the coating does not have optimum uniformity and structure. This situation prevails when a highly refractory material, such as tungsten, or carbon is used.

An object of this invention is to provide a method for depositing an improved, uniformly coherent and adherent, dense coating of chemical elements and chemical compounds of controlled thickness upon any suitable substrate surface employing a plasma forming fluid consisting of a mixture of monatomic and diatomic gases.

Another object of this invention is to provide a method for depositing an improved, uniformly coherent and adherent, dense coating of pyrolytic carbon and refractory carbides upon suitable substrate surfaces for high temperature applications on any size or shape of substrate surface by employing a plasma forming fluid consisting of a mixture of a monatomic and a diatomic gas.

Other objects of this invention will, in part, be obvious and will, in part, appear hereinafter.

In order to more fully understand the nature and objects of this invention, reference should be had to the following detailed description and drawings in which:

FIG. 1 is a cross-sectional view of the plasma jet generator employed in producing pyrolytic coatings by a plasma jet technique embodying the teachings of this invention;

FIG. 2 is a cross-sectional view of an improved pyrolytic coating of material on a surface of a substrate; and

FIG. 3 is a view, partly in cross-section, showing the method of depositing an improved pyrolytic coating of a material employing another plasma jet technique embodying the teachings of this invention.

In accordance with the teachings of this invention and in the attainment of the foregoing objects, there is provided an improved coating of dense, uniformly coherent and adherent pyrolytic carbon such, for example, as carbon in the form of graphite, on a suitable substrate. The pyrolytic coating of carbon has a bulk density of from 2.1 to 2.25 grams per cubic centimeter and an impurity content of less than 20 parts per million.

A preferred method for depositing the improved coating of carbon is to introduce one or more suitable chemical elements and chemical compounds, in the form of a gas or a low boiling point fluid, into an ionized plasma-forming fluid or plasma jet.

This preferred method permits a more uniform introduction of a reactant material at a predetermined, controlled rate into a plasma jet.

Excellent results are obtained when a pyrolytic carbon coating is formed on a carbon substrate by utilizing aliphatic and aromatic halides of carbon. Examples of suitable aliphatic halides are tetrachloromethane, tetrabromomethane, trichloromethane, tribromomethane, dichloromethane, dibromomethane, monobromomethane, monochloromethane, monobromoethane, monochloroethane, monobromopropane and the like. Suitable aromatic halides are monochlorobenzene, monobromobenzene, dichlorobenzene, dibromobenzene, chlorotoluene, bromotoluene and the like.

A plasma-forming fluid consisting of a monatomic gas and at least one other gas having a diatomic molecule has proven to be very satisfactory in producing the improved pyrolytic coating of carbon. A suitable plasma-forming fluid comprises argon gas as the monatomic gas and hydrogen gas in quantities up to 10 mole percent as the diatomic gas.

Hydrogen is chosen as the diatomic gas ingredient because of its high internal energy and its high affinity for halides. The amount of hydrogen present in the plasma jet is always many times greater than that required for the reaction in the carbon carrying reactant material introduced into the ionized plasma-forming fluid. Depending on the reactant material, a chemical reaction occurs between the hydrogen gas and the reactant material, or chemical dissociation of the reactant material occurs in the plasma-forming fluid, producing carbon which is then deposited as the improved pyrolytic coating. Other reactant products are carried off as a gas.

The amount of contaminants in the improved pyrolytic carbon coating resulting from a process embodying the teachings of this invention is only 20 parts per million maximum.

With reference to FIG. 1, there is shown a plasma jet generator 10 suitable for depositing the improved pyrolytic coating of carbon on a suitable substrate material.

The plasma-jet generator is comprised of an arc chamber 12 and a product chamber 14.

The arc chamber 12 is defined by a circular metal wall 16 having an outwardly extending integral metal peripheral flange 18 at one end and is enclosed by an anode 20 disposed at one end of the wall 16 and a back plate 22 disposed at the other end of the wall 16. The wall 16 is made of brass and contains an integral coolant passage 24 for the circulation of a coolant such, for example, as water.

A plasma fluid inlet tube 26 passes through the wall 16 and into the arc chamber 12. The plasma fluid inlet tube 26 permits the plasma-forming fluid to be introduced directly into the enclosed arc chamber 12.

The wall 16 is joined to the anode 20 by disposing the peripheral flange 18 into a recessed portion 28 of an integral peripheral flange 30 of the anode 20. The flanges 18 and 30 may be secured by any suitable mechanical means.

A gas tight seal 32 between the wall 16 and the anode 20 is obtained by employing an O-ring type seal 32. The seal 32 is disposed in an annular groove 34 of the flange 30.

The anode 20 contains an integral passage 36 for the circulation of a coolant such, for example, as water and has an axially disposed funnel shaped bore 38. The bore 38 has an entrance 40 and an exit 42. The diameter of the entrance 40 is greater than the diameter of the exit 42.

A reactant inlet tube 44 passes completely through the anode 20 and enters into the bore 38. The reactant inlet tube 44 is disposed perpendicular to the axis of the bore 38. The reactant inlet tube 44 permits reactant material to be introduced into the plasma jet stream beyond the arc column.

An insert 46 is disposed within the bore 38. In producing pyrolytic carbides and pyrolytic carbon the insert 46 is made of carbon in the form of graphite. The insert 46 prevents the erosion of the anode 20 during the operation of the generator 10 and thereby prevents any brass from contaminating the

pyrolytic coating of material which is formed. An outwardly extending flange 48 is seated within a recess 50 of the bore 38 to permit a flush contour surface within the bore 38. A hole 52 permits the insertion of the reactant inlet tube 44 through the insert 46 and into the bore 38.

The back plate 22 is made of brass and is joined to the wall 16 by suitable mechanical means. A gas tight seal is achieved by disposing an annular gasket 54 of an electrically insulating material between the back plate 22 and the wall 16. The back plate 22 has an axially disposed raised embossment 56.

A cathode holder 58 is disposed through an aperture 60 in the embossment 56. A gas tight seal is achieved between the holder 58 and the back plate 22 by an O-ring type gasket 62 disposed in an annular groove 64 within the aperture wall 66.

The cathode holder 58 is made of silver plated brass. The holder 58 has an integral passageway 68 to permit the circulation of a coolant, such, for example, as water. The holder 58 also has a recessed means 70 for supporting a cathode 72 inserted therein.

The cathode 72 is made of a material selected from the group consisting of carbon, tungsten, tantalum, molybdenum and alloys thereof.

Since ablation of the cathode 72 is a natural occurrence during the operation of the generator 10, carbon in the form of graphite is a preferred material for making the cathode 72 used in pyrolytically depositing coatings of carbon and carbides.

The product chamber 14 is made of silver plated brass and is joined to the anode 20 by suitable means. The product chamber 14 is where the pyrolytic coatings of this invention are deposited on suitable substrates. A viewing port 74 in a wall 76 of the chamber 14 permits one to have easy access for measuring the temperature of a substrate surface as well as allowing a means for locating a substrate properly in respect to the stream of the plasma flame.

The plasma-forming fluid consisting of argon gas with up to 10 mole percent of hydrogen gas is introduced into the enclosed arc chamber 12 through the plasma fluid inlet tube 26. A preferred range for the plasma-forming fluid comprises argon gas containing from 0.8 mole percent of hydrogen gas to 3.8 mole percent of hydrogen gas. The plasma-forming fluid has a gas flow rate of from 0.8 gram-moles per minute to 3.0 gram-moles per minute. A preferred flow rate is 1.25 grams-moles per minute.

The plasma jet generator arc current range is between 200 amperes and 1,000 amperes.

At the preferred gas flow rate of 1.25 gram-moles per minute, a plasma-forming fluid comprised of argon gas containing 3.8 mole percent of hydrogen gas, when ionized by an arc current of 300 amperes, has a specific enthalpy of 56 Kilocalories per gram-mole of the plasma-forming fluid. This is equivalent to a temperature of approximately 9,400° K.

A substrate 78, such, for example, as carbon in the form of graphite, is disposed within the product chamber 14 at a distance of from 2 to 5 centimeters from the exit 42 of the axial bore 38 of the anode 20. A preferred distance for disposing the substrate 78 is to place it 3 centimeters in front of the exit 42 of the axial bore 38.

The ionized plasma-forming fluid heats a surface 80 of the substrate 78 to an elevated temperature. It is upon this heated surface 80 that a pyrolytic coating, in this instance carbon, is deposited.

Since normal operation of the plasma jet generator 10 produces an ionized plasma-forming fluid, or plasma jet, having a temperature of approximately 9,400° K. at the exit 42 of the bore 38, the temperature of the surface 80 of the substrate 78 heated by the plasma jet will vary from approximately 1,200° to 3,000° K. At the optimum positioning of the substrate 78 in the product chamber 14, the average temperature of the surface 80 is approximately 2,500° K.

The substrate 78 is heated directly by the plasma jet, and not from an external source. Any size or shape of substrate 78 may be coated by methods embodying the teachings of this in-

vention. The substrate 78 may be moved in any direction within a plane perpendicular to the centerline axis of the plasma jet discharge and so obtain a uniform coating over a large area of the surface 80 of the substrate 78.

Conversely, the substrate 78 may be held stationary and the plasma jet programmed to direct its discharge over the changing surface 80. Irregularly shaped, and sizes of, substrates may also be programmed accordingly in order to achieve a uniform coating over the entire surface 80 of the substrate 78.

In choosing the proper reactants for the desired end product to be produced, one has to know the enthalpy change of the chemical reaction or dissociation which will occur in the plasma jet, the enthalpy of the plasma-forming fluid and the internal energy to be expected within the plasma jet. It is most desirable that the required reactants are introduced at that given rate which is sufficient to allow the internal energy of the plasma jet to supply the necessary heat of reaction or dissociation to carry all expected chemical reactions or dissociations to completion. Therefore, depending upon the heat of reaction or dissociation of the expected chemical reactions or dissociations and employing the teachings of this invention, reactants can be introduced into the plasma jet at rates up to 10 gram-moles per hour.

With added reference to FIG. 2 there is shown a pyrolytically coated substrate 100. The pyrolytically coated substrate 100 consists of a carbon substrate 102 and a layer 104 of dense, coherent and adherent pyrolytic carbon disposed on a surface 106.

One or more of the aliphatic and aromatic halides of carbon is introduced into the plasma jet generator 10 through the reactant inlet tube 44 at a rate of from 0.01 gram-mole per minute to 0.2 gram-mole per minute. The optimum flow rate is 0.1 gram-mole per minute.

The layer 104 of improved dense, uniformly coherent and adherent pyrolytic carbon is deposited upon the heated surface 106 of the carbon substrate 102 at a rate of between 0.05 grams per minute to 1.0 grams per minute. An average deposition rate of 0.1 grams per minute is equivalent to a thickness of 0.005 inch of pyrolytic carbon being deposited on 2 square centimeters of substrate 102 per minute. Compared to previously known conventional methods, this is a substantial increase in the plating or coating of a substrate with a pyrolytic carbon.

The layer 104, or pyrolytic coating, of carbon deposited is extremely dense when compared to commercial graphite known previously to those skilled in the art and has a density of from 2.1 to 2.25 grams per cubic centimeter. Being a more uniform coating, the improved pyrolytic coating 104 of carbon affords great reliability for high temperature applications in the aeronautical industries and similar endeavors. A particular application of this improved pyrolytic coating 104 of carbon is in the design of rocket propulsion system nozzles and in the throat sections of the venturi portion of a rocket engine.

Refractory carbides are also deposited upon suitable substrates, such as carbon, tungsten, molybdenum and the like, utilizing the same process as heretofore disclosed for the production of pyrolytic carbon. A mixture of volatile compounds of the metal and carbon is used as the reactant fluid for the preparation of the refractory carbides by the plasma jet technique. This process also employs a mixture of monatomic and diatomic gases such, for example, as helium and

hydrogen, helium and nitrogen, argon and hydrogen and argon and nitrogen, as a plasma-forming fluid.

The reactants decompose in the plasma jet and the dissociated elements react with one another to form the required carbide which is transported by the plasma jet fluid to be deposited upon a substrate surface in a dense, uniformly coherent and adherent pyrolytic coating. The halide of the reactant gas is exhausted from the plasma jet generator.

Suitable reactant metal compounds for forming refractory carbides by the embodiments of the teachings of this invention are the compounds of metal and metallic halides. These metal-

75

lic halides include halides of silicon such for example, as trichlorosilane, silicon tetrachloride, silicon tetrabromide, chlorides of boron, aluminum, titanium, zirconium, molybdenum and tungsten, as well as the bromides of boron, aluminum, titanium, zirconium, molybdenum and tungsten. Suitable carbon reactants are the same as those used in the depositing of pyrolytic carbon embodying the teachings of this invention.

Employing solid chemical compounds with low sublimation and decomposition temperatures, it has been found that metal carbonyls selected from a group of metals consisting of tungsten, chromium, molybdenum, iron, cobalt, nickel, rhodium, iridium and osmium are the most suitable for depositing pyrolytic coatings of metal carbides upon suitable substrates utilizing the plasma jet technique. The metallic carbonyls decompose into a metal and carbon monoxide at relatively low temperatures such, for example, as tungsten, carbonyl, molybdenum, carbonyl and chromium carbonyl, all of which decompose without melting at approximately 150° C.

The metallic carbonyls are reacted with aliphatic and aromatic carbon halides in a plasma-forming fluid comprising a mixture of monatomic and diatomic gases, such, for example as a mixture of argon and hydrogen containing up to 10 mole percent of hydrogen, resulting in a uniformly dense, coherent and adherent pyrolytic coating of a metallic carbide upon the surface of a suitable substrate. The same aliphatic and aromatic carbon halides hereinbefore described as reactants with metallic halides for the production of metallic carbides embodying the teachings of this invention are suitable reactant materials.

Other suitable reactant materials for obtaining metallic carbide coatings upon suitable substrate surfaces are found in the group of metallo-organic compounds. These metallo-organic compounds yield a metal carbide upon thermal decomposition without the plasma jet. The metal carbide coating is produced by the same general plasma jet methods hereinbefore described by the teachings of this invention.

It has been found that each of the metallo-organic compounds of methyltrichlorosilane and aluminum triethyl yield respective pyrolytic coatings of silicon carbide and aluminum carbide. Other suitable metallo-organic compounds which yield aluminum carbide are trialkylaluminum, tri-n-propylaluminum, tri-n-butylaluminum, tri-i-propylaluminum and di-isobutyl-aluminum hydride.

Other chemical elements and chemical compounds are deposited on suitable substrate surfaces using the plasma jet technique embodying the teachings of this invention. When molybdenum carbonyl and hydrogen sulfide are used as the reactants in a plasma-forming fluid comprising argon and hydrogen, the resulting deposit of molybdenum sulfide deposited on a graphite substrate was found to be both coherent and adherent as well as uniformly dense throughout its structure.

Employing the embodiment of the teachings of this invention, uniformly dense, coherent and adherent coatings of chemical compounds such as oxides, carbides, borides and silicides are also feasible.

With reference to FIG. 3 there is shown another means of depositing a dense uniformly coherent and adherent coating 150 of chemical elements and chemical compounds on a surface 152 of a suitable substrate 154. This means utilizes the plasma jet generator 10 of FIG. 1 as a means to heat the surface 152 with an ionized plasma-forming fluid 156 and impinge reactant material 158 upon the heated surface 152.

While the ionized plasma-forming fluid 156 continues to heat the surface 152 of the substrate 154, the reactant material 158, in a gaseous form, is caused to impinge upon the heated surface 152. In one instance the reactant material 158 chemically reacts with the ionized plasma-forming fluid 156 to produce the required material for the coating 150. Any other chemical products resulting from the chemical reaction passes off as a gas.

A second possible reaction which the reactant material 158 may undergo is to chemically decompose upon impinging with the heated surface 152 instead of chemically reacting with the ionized plasma-forming fluid 156. Upon chemically decomposing, the required material for the coating 150 is deposited on the surface 152 and the remaining portion of the decomposed reactant material 158 passes off as a gas.

The reactant material 158, in a gaseous form, flows through a reactant tube 160 which controls its direction of flow. The direction of flow of the gaseous reactant material 158 is such that the theoretical centerlines of travel of the reactant material 158 and the ionized plasma-forming fluid 156 will intersect on the surface 152 of the substrate 154 where the layer 150 of pyrolytic material will be deposited.

The reactant inlet tube 160 is made of a suitable material, such, for example, as glass, metal and the like. The material is one that is inert to the reactant material 158 which is flowing through the tube 160. Although the tube 160 must be disposed close enough to the surface 152 to assure proper impingement of the reactant material 158 thereon, the heat is not sufficient to have any deleterious effects on the tube 160.

The reactant material 158 flows at a sufficient velocity to overcome the effects occasioned by the velocity of the ionized plasma-forming fluid 156 impinging on the surface 152 of the substrate 154.

With both the ionized plasma-forming fluid 156 and the reactant material 158 impinging the surface 154 in the same area, good mixing of them will occur. Therefore, should the reactant material 158 be a material that will chemically decompose to form the layer 150, a good thermal transfer energy is obtained to accomplish the required chemical decomposition. If the reactant material 158 is a material that will chemically react with a portion of the ionized plasma-forming fluid 156, the mixing of the reacting components is easily accomplished.

In either instance, the resulting required material desired for the pyrolytic layer 150 is deposited on the surface 152. Any other chemical products resulting from either the chemical decomposition, or the chemical reaction, of the reactant material 158 is exhausted by suitable means from the surface 152 as a gas as the velocity of the reactant material 158, is sufficient to aid the flow of gaseous products away from the surface 152 as well as being able to overcome the effects of the velocity of the ionized plasma-forming fluid 156.

The following examples are illustrative of embodiments of the teachings of this invention.

#### EXAMPLE I

Embodying the teachings of this invention pyrolytic carbon was deposited by the plasma jet technique upon a carbon substrate using chloroform as a reactant material. The arc current for the plasma jet was 300 amperes. The specific enthalpy of the plasma jet was 56 kcal/gram-mole or a temperature approximately 9,400° K. The graphite substrate was disposed 3 centimeters from the plasma jet nozzle and its surface temperature was approximately 2,500° K. as a result of heating from the plasma jet. The reactant fluid of chloroform was introduced into the plasma jet through an inlet tube in the nozzle at a rate of 0.1 gram-mole per minute. The anode nozzle and the cathode of the plasma jet generator were made of high purity carbon in the form of graphite.

The plasma-forming fluid consisted of argon gas containing 3.8 mole percent of hydrogen gas. The plasma-forming fluid was introduced into the plasma jet generator at a gas flow rate of 1.25 moles per minute.

The resulting pyrolytic carbon was deposited upon the carbon substrate at an average rate of 0.1 gram per minute and had a bulk density of 2.1 to 2.25 grams per cc. The resulting pyrolytic carbon had the same structure as pyrolytic carbon produced by previously known methods of the art as determined by X-ray diffraction patterns. The impurity content of the pyrolytic carbon was less than 20 ppm as determined by

spectroscopic analysis. Microscopic examination of the interface between the substrate surface and the pyrolytic carbon showed a very coherent and adherent structure.

## EXAMPLE II

Embodying the teachings of this invention silicon carbide was deposited by the plasma jet technique upon a surface of a graphite substrate using a mixture of trichlorosilane and propylene as the reactants. The arc current employed in the plasma jet generator was 300 amperes. The specific enthalpy of the plasma jet was 56 kcal/gram-mole or a temperature approximately 9,400° K. A graphite substrate was disposed 4 centimeters from the plasma jet nozzle and the substrate surface temperature was approximately 1,600° C. as a result of heating from the plasma jet. The mixture of reactants was introduced into the plasma jet at a rate of 0.4 gram-moles per hour for propylene and 2.0 grams-moles per hour for the trichlorosilane.

The plasma-forming fluid consisted of argon gas containing 3.8 mole percent of hydrogen gas. The plasma-forming fluid was introduced into the plasma jet generator at a gas flow rate of 1.25 moles per minute.

A deposit of dense uniformly coherent and adherent silicon carbide was deposited on the graphite substrate at a rate of 0.15 grams per minute. Upon examination, the structure of the silicon carbide was found to be cubic.

## EXAMPLE III

Embodying the teachings of the invention a coating of molybdenum sulfide was deposited by the plasma jet technique upon a graphite substrate, disposed 5 centimeters from the plasma jet nozzle, using a reactant mixture of molybdenum carbonyl and hydrogen sulfide gas. The arc current for the plasma jet generator was 300 amperes. The plasma-forming fluid consisted of argon gas containing 3.8 mole percent of hydrogen gas. The plasma-forming fluid was introduced into the plasma jet generator at a gas flow rate of 1.25 moles per minute. The specific enthalpy of the plasma jet was 52 kcal/gram-mole or a temperature of approximately 9,300° K. The graphite substrate had a surface temperature that was approximately 1,300° K. as a result of heating from the plasma jet. The reactant mixture of molybdenum carbonyl and hydrogen sulfide was introduced into the plasma jet through an inlet tube in the nozzle at a rate of 0.5 gram-moles per hour for molybdenum carbonyl and 2 gram-moles per hour for the hydrogen sulfide. The anode nozzle and the cathode of the plasma jet generator were made of copper and tungsten, respectively.

The resulting deposit of molybdenum sulfide was deposited upon the surface of the graphite substrate at a rate of 0.3 grams per minute.

Suitable substrate materials which can be used in conjunction with the teachings of this invention are dependent upon the end use of the resulting product. Carbon, in the form of graphite, is the most convenient substrate to employ since the coated substrate has a more universal end use. However, coatings of refractory carbides can also be deposited on the respective metals employed in the refractory carbides, such as tungsten for tungsten carbide, molybdenum for molybdenum carbide and the like. Other suitable substrates are iron, cobalt, nickel, rhenium, osmium, chromium, boron, aluminum, zirconium and titanium.

In employing the impingement technique for depositing the coating 150 of chemical elements and chemical compounds, the same reactants disclosed in the preferred method, as well as the same type of plasma-forming fluid, the same plasma generator and the same operating conditions is utilized. Again, suitable substrates to be employed will be dependent upon the end use of the resulting product.

This method is similar to the pyrolytic coating process in which the substrate is heated by resistance or inductive heating. The technique of heating a surface of a substrate with an ionized plasma-forming fluid is more flexible however.

While the invention has been described with reference to particular embodiments and examples, it will be understood, of course, that modifications, substitutions and the like may be made therein without departing from its scope.

I claim as my invention:

1. A process for producing a pyrolytic coating on a surface of a substrate comprising:
  1. introducing a plasma-forming fluid into a plasma jet generator at a gas flow rate of from 0.8 gram-moles per minute to 3.0 gram-moles per minute, said plasma-forming fluid consisting of a mixture of argon and from 0.8 to 10 mole percent of hydrogen,
  2. ionizing said plasma-forming fluid with an electrical current of from 200 to 1,000 amperes,
  3. introducing a reactant material consisting of a mixture of molybdenum carbonyl and hydrogen sulfide into said ionized plasma forming fluid whereby said reactant material undergoes a chemical change within said ionized plasma-forming fluid to form a reaction product of molybdenum sulfide which is transported by said ionized plasma-forming fluid to a substrate where at least a portion of said reactant product is deposited on a heated surface of said substrate in a dense, uniform, coherent and adherent coating.

\* \* \* \* \*